

Sept. 6, 1932.

E. A. VAZQUEZ

1,876,522

RECOVERY OF BY-PRODUCTS OF SUGAR EXTRACTION

Filed Oct. 31, 1930



Inventor  
Eugenio Antonio Vazquez.

384  
Pennie, Davis, Marvin & Edmonds  
Attorneys

## UNITED STATES PATENT OFFICE

EUGENIO ANTONIO VAZQUEZ, OF HABANA, CUBA, ASSIGNOR TO VAZCANE PROCESS, INC., A CORPORATION OF DELAWARE

## RECOVERY OF BY-PRODUCTS OF SUGAR EXTRACTION

Application filed October 31, 1930. Serial No. 492,547.

This invention relates to a process for the treatment of sugar cane and of the components derived therefrom, by which there is produced sugar and fiber pulp as the main products, and volatile organic compounds as by-products.

It is customary in the process of isolating the sugar contained in sugar cane to pass the cane through a series of heavy crushing mills or rolls, either as received at the mill or previously cut or shredded. The juice or sugar bearing liquids are extracted or expressed from the plant tissues by means of heavy pressure exerted by the crushing rolls. These rolls are of cast iron, weighing as high as fifteen tons each, and the cane is passed successively through several sets of such rolls adjusted progressively closer together.

Between the successive sets of rolls it is customary to add dilute juice from the set of rolls next in line (or water as maceration or imbibition water) for the purpose of obtaining a higher extraction of the available sucrose. From the last roll the woody refuse of the cane, called bagasse or megasse, is delivered containing approximately 50% moisture and in the state of small fiber aggregates. The fibers are not individually separate, but are still bound together in bundles by the binding or cementitious materials in the cane.

The customary method of disposal of the bagasse or waste refuse is as fuel for a source of power for the sugar mills. In recent years, however, due to the diminishing supply of forest wood, other sources of supply of fiber pulp for paper making have been exploited, and bagasse has been the subject of a considerable amount of experimenting. Bagasse has been used in the production of insulating wallboard, but its physical state in such a wall-board is that of dry grass or hay, rather than that of paper pulp. However, the use of sugar cane as a raw material from which to manufacture mechanical paper pulp has recently been accomplished by a process set out in Letters Patent No. 1,688,904, granted to me October 23rd, 1928.

In this process the cane is separated, by

grinding or abrading it, into individual fibers or aggregates of relatively few fibers, smaller than have ever been produced by any prior methods of sugar recovery. The sugar is removed, or obtained, from this material by a method such as diffusion. The comminuted material is dispersed in a solvent bath, in which it is agitated until the solvent is thoroughly worked into the fibers. The solvent is then separated from the comminuted cane and the latter redispersed in a second bath. In this bath the material is again agitated in the same manner as in the first, after which it is again separated. These steps of dispersing, agitating and separating are repeated as often as is necessary to complete the separation of sugar from the cane.

Water is used as the solvent only in the last dispersing treatment. Prior to the last treatment the solvent is the dilute sugar solution from a subsequent dispersing stage. In other words, the solvent is circulated countercurrent to the cane, fresh water being added to the final bath, and the solution from each bath becomes the solvent liquid for another bath until it is removed from the first bath as concentrated sugar solution and delivered to the sugar boiling house.

The pulp resulting from the application of the process of my Patent No. 1,688,904 is much finer and much more uniform than ordinary bagasse, but can be used equally as well as ordinary bagasse for the production of fiber pulp according to my present invention.

My present invention is a process whereby the bagasse, from which the sugar has been removed, is so treated as to obtain therefrom fibers whose chemical composition and physical state differ from the original fiber in such a way that the fiber is suitable for use in the manufacture of wall-board, corrugated board, wrapping paper, newsprint paper, higher grades of paper or any other paper product, and also to obtain from the bagasse other products of commercial value which are contained therein or chemically formed therefrom. This process is applicable both to the usual sugar mill process whereby the cane is shredded or torn and the juice then

removed by crushing, and to the process set forth in my previous patent referred to above.

In the usual sugar mill practice a sugar mill operates for only a few months out of the year and for the remaining part of the year the sugar mill remains inactive. My new process is so carried out that the bagasse taken from a sugar mill during the active period is stored in treating tanks where it undergoes one of the steps necessary in its treatment while the sugar mill is finishing its period of active operation. This step consists of the treatment of the bagasse by storing it in large vats or tanks and completely covering it with a dilute lime solution. The solution is allowed to remain in contact with the bagasse for a period of time sufficient for it to react with the binding or cementitious materials which hold the fibers together in fiber bundles, and to dissolve or extract these materials from the bagasse. This is usually accomplished in a period of from three to four months or even less, depending upon the concentration of the lime solution and local conditions.

In the ordinary processes for the production of fiber pulp from bagasse or other woody material, the material is submitted to a digestion usually under heat and pressure with certain alkalies. In order to remove completely the incrusting matter, the time of cooking, the pressure and strength of alkali have to be adjusted for digesting or cooking the hardest parts of the fiber. This treatment is too drastic for the finer or weaker parts of the fiber, and consequently the yields are low.

In the process of the present invention the action is very mild, the time for reaction is considerable and the yield is therefore substantially great as compared with the cooking process. By the time the incrusting materials have been removed from the bagasse, the sugar mill has finished its normal operation and has become inactive. Its equipment therefore becomes available for the further steps of my process. The bagasse pulp which has been in storage may be freed from the lime solution by passing it through the cane mills using imbibition water for washing, the same as the cane was originally treated for the removal of sugar, or the bagasse pulp may be passed through a dispersing, agitating and screening system with a counter-flow system such as disclosed in my prior patent mentioned above. By this treatment the pulp and liquid are mechanically expressed or agitated, so as to free completely the fibres of the pulp and to leave in the lime solution the cementitious or binding materials which have been rendered soluble.

The fibrous pulp may be dried after the removal of the lime solution, or may be bleached or subjected to a beating and refin-

ing operation and lapped, or may be used directly in the manufacture of paper.

I have obtained yields of 55% of unbleached pulp on the basis of dry Cuban bagasse employed, and of 44.7% of bleached pulp on the basis of dry Cuban bagasse employed. The lime solution remaining after the removal of the pulp is passed on through the settling tanks or filters of the sugar mill, where the sludge which has formed therein is removed. This sludge contains a large part of the lime which is used in the treatment of the bagasse in the form of phosphoric or organic acid salts, together with a certain amount of humus-like material. This sludge may be treated by burning to recover the lime, or may be used directly as fertilizer. Another possible use for this sludge lies in the recovery of the organic salts of calcium as such. It is obvious that still other treatments may be used to recover the valuable components in still different combinations.

The liquid from the filters is passed on into the evaporators of the sugar mill. With slight changes in these evaporators they may be converted to function as fractionating stills and the lime solution may be fractionated so as to recover the volatile compounds formed from the bagasse. Such volatile compounds vary in kind and quantity, depending upon the strength of the lime solution used and the time of treatment. After the volatile organic constituents of this lime solution have been recovered, the liquor may be further treated to obtain all or a part of the soluble solids it contains.

A flow sheet which forms a part of this description shows in diagrammatic form the steps of this process and may be referred to in connection with the following detail description of the operation of this process.

As shown at the left of the flow sheet the untreated cane is first subjected to a shredding or tearing treatment in what is ordinarily a crusher or hammer mill. After this treatment the cane is subjected to the crushing action of the sugar mill proper, wherein the heavy crushing rolls express the saccharine juices from the cane. During this treatment water is usually added to complete the removal of the sugar.

The course of the cane in receiving this treatment is shown by the full line starting with the untreated cane and passing through the steps of shredding or tearing and of crushing. It will be noted that water is indicated as being added at the crushing step. This is customary although not absolutely essential.

An alternate method of treating the cane is shown in dotted lines on the flow sheet. This is the method disclosed in my patent already referred to and consists in grinding the untreated cane, dispersing it and agitating

ing it in water. This dissolves the sugar juices which are then removed by straining or screening.

Although the crushing and screening and the dispersing and agitating and screening or straining are shown, but once on the flow sheet, it is obvious that these steps and the other steps of the process as well may be repeated several times in order to make the treatment of the cane complete.

The two alternate processes shown differ only up to the point where the fibers are screened or strained from the aqueous suspension, and the flow sheet shows only one process from this point on.

The fibrous material from the last roll of the crushing mill is commonly known as bagasse. The bagasse is generally considered as practically free from sugar but usually contains a small quantity, and contains about 50% moisture. The individual fibers of bagasses are bound together by the cementitious material therein. This material contains the lignin and the pentosan constituents of the cane. The juice expressed by the mills or removed from the dispersing tanks passes into settling tanks where it is treated with lime and the foreign matter therein allowed to settle out. It usually then passes through filters where the last particles of foreign matter, fibers, sludge, etc. are removed.

From the filters the sugar solution passes into the usual evaporators where it is evaporated and the sugar crystallized.

The parts of the process set out above is that of the usual sugar extraction process and is intended to be described merely as a basis upon which to build the following process which is my invention. The process referred to above being the usual sugar process, it is obvious that changes known in the art and modifications of this process may be made without departing from the spirit of my invention.

My invention comprises the superimposing of the following process on to the usual sugar making process, and this added process is shown by the double lines which start with the bagasse taken from the expressing mills in the usual sugar process.

The bagasse from the usual sugar process is placed, according to my process, in large vats or tanks where it is covered with a solution of lime and allowed to remain for a sufficient time for the lime to react with the constituents of the bagasse, which bind the individual fibers together, sufficiently to loosen these fibers. The particular solution which I have found preferable is a solution containing approximately 5% to 10% of lime based on the dry weight of the fiber. The bagasse is preferably allowed to remain completely covered with lime solution for a prolonged period, usually about three or four

months. The tanks may be covered to prevent evaporation. The long period of storage not only allows the lime to react properly with the bagasse, but also provides time in which the sugar mill may finish its season's work of isolating sugar and thus have its equipment available for use in the treatment of the bagasse. The bagasse and lime solution are fed either to the crushing or dispersing and agitating equipment, depending upon which the two processes is in use in the sugar mill. After whichever of these two treatments is used the bagasse and lime solution is screened or strained. The agitation received either in the crushing or in the dispersing and agitating treatment completely frees the fibers which have already been loosened by the action of the lime solution on the cementitious constituents. Thus, when the screening or straining takes place a fibrous pulp is removed (as shown by the double lines on the flow sheet) which is suitable for further treatment such as bleaching, etc., and which may be subsequently used in the manufacture of paper goods of almost any desired class.

The liquid from the screening or straining is conveyed to the settlers where the sludge therein is allowed to settle out. The liquid is then filtered if required. The sludge which settles from the liquid at this time contains a large part of the lime used in the treatment of the bagasse. This material is usually in the form of salts of phosphoric and organic acids. Various methods may be used for the recovery of the valuable constituents of this sludge. The sludge may be burned whereby the lime is recovered, or it may be used directly as fertilizer where it has particular value because of its nitrogen and phosphorous content. The nitrogen is acquired from the bagasse during the treatment thereof. The organic salts may also be recovered as such.

The resulting clear liquid is conducted (as shown by the double lines) to the evaporating or fractionating apparatus. In using this process the evaporators used in the normal sugar process are converted by making some minor changes so that they will function to fractionate this liquid. From this fractionation various volatile organic compounds are obtained. The liquor may be further treated for the recovery of the soluble solids it contains.

On the flow sheet the usual steps in the process of extracting and isolating sugar are shown as rectangular blocks and the usual course of materials passing through such a process is shown by a single line. An alternate process such as described in my prior Patent No. 1,688,904, granted to me October 23rd, 1928, is shown in dotted lines. The materials fed into the process and taken from the process at various stages are shown in

circles. Thus, in the usual sugar process untreated cane passes through the shredding or tearing step through the crushing step in which the water is added; the juice flows to the screening or straining step while the bagasse is taken to be used as fuel under the boilers, and the juice continues to the settling and filtering step from which foreign material is discarded and through the evaporating step from which sugar is taken.

The steps added by my improved process are shown on the flow sheet enclosed in octagon shaped boxes, and the flow of material through these steps and their return through certain steps in the usual sugar process are shown by double lines which start from the bagasse and run through the crushing or through the dispersing and agitating step to the screening or straining step and on. The products produced by this process are shown below the steps of the process, and are the fibrous pulp, sludge, volatile organic compounds and the soluble solids of the mother liquor, etc., and the products which may be produced from these materials.

I claim:

1. The process of extracting sugar from sugar cane and recovering byproducts therefrom which consists in extracting sugar from cane in the usual manner, storing the bagasse derived from this extraction in a solution of lime until the normal period of operation of the sugar mill is completed and returning the bagasse and treating liquor to the sugar mill and subjecting it to treatment therein analogous to that of the sugar extraction process to obtain fiber, pulp and other byproducts therefrom.

2. The process of preparing bagasse for the recovery of by-products and fibers which comprises immersing the bagasse in a dilute solution of lime at normal temperature for a sufficient length of time to loosen the fibers therein.

3. The process of preparing bagasse for the recovery of by-products and fibers which comprises treating the bagasse at normal temperature with a solution containing a weight of lime equal to approximately 5% to 10% of the weight of the air-dry fibers to liberate the fibers therein.

4. The process of preparing bagasse for the recovery of by-products and fibers which comprises immersing the bagasse in a dilute solution of lime at normal temperature for a sufficient length of time to loosen the fibers therein and subjecting the solution and fibers to light mechanical agitation to complete the freeing of the fibers.

5. The process of recovering by-products and fibers from bagasse which comprises immersing the bagasse in a dilute solution of lime at normal temperature for a sufficient length of time to loosen the fibers therein, subjecting the solution and fibers to light me-

chanical agitation to complete the freeing of the fibers and separating the solution from the fibers.

6. The process of recovering by-products and fibers from bagasse which comprises immersing the bagasse in a dilute solution of lime at normal temperature for a sufficient length of time to loosen the fibers therein, and separating the solution from the fibers.

7. The process of recovering by-products and fibers from bagasse which comprises immersing the bagasse in a dilute solution of lime at normal temperature for a sufficient length of time to loosen the fibers therein and separating the solution from the fibers by counter-current washing.

8. The process of recovering by-products from bagasse which comprises treating the bagasse with a dilute solution of lime at normal temperature and over a considerable period of time, separating the solution from the fibers and distilling from the solution the products extracted from the bagasse.

9. The process of recovering by-products from bagasse which comprises treating the bagasse with a solution of lime at normal temperature for a sufficient length of time to loosen the fibers therein and recovering from the alkaline solution products extracted from the bagasse.

10. The process of recovering by-products from bagasse which comprises immersing the bagasse in a dilute solution of lime at normal temperature for a sufficient length of time to loosen the fibers therein, subjecting the bagasse to light mechanical agitation to completely free the fibers, separating the solution from the fibers and separating the sludge from the solution.

11. The process of recovering by-products from bagasse which comprises immersing the bagasse in a dilute solution of lime at normal temperature a sufficient length of time to loosen the fibers therein, separating the solution from the fibers and separating the sludge from the solution.

12. The process as defined in claim 11 in which the sludge is separated from the solution by settling and filtering.

13. The process of recovering by-products from bagasse which comprises immersing the bagasse in a dilute solution of lime at normal temperature for a sufficient length of time to loosen the fibers therein, subjecting the bagasse to light mechanical agitation to completely free the fibers, separating the solution from the fibers, separating the sludge from the solution, and recovering the products extracted by the solution.

14. The process of recovering by-products from bagasse which comprises immersing the bagasse in a dilute solution of lime at normal temperature for a sufficient length of time to liberate the fibers therein, separating the solution and fibers and removing a portion of

the materials extracted from the bagasse as solids and distilling the remainder.

15. The process of recovering by-products from bagasse which comprises immersing the bagasse in a dilute solution of lime at normal temperature for a sufficient length of time to liberate the fibers therein, separating the solution from the fibers, distilling from the solution a portion of the products extracted 10 from the bagasse, and recovering other products extracted from the bagasse as alkaline organic salts.

16. The process of recovering by-products from bagasse which comprises covering the bagasse with a dilute solution of lime, allowing it to stand so covered for several months at normal temperatures, subjecting the solution and fibers to light mechanical agitation, separating the solution from the fibers by 20 counter-current washing, and straining, settling and filtering the solution, burning the sludge thus obtained to recover the lime therein and fractionally distilling the filtered solution to obtain furfural and vanillin.

25 In testimony whereof I affix my signature.  
EUGENIO ANTONIO VAZQUEZ.

30

35

40

45

50

55

60

65